

Patented May 1, 1923.

1,453,289

# UNITED STATES PATENT OFFICE.

EDWARD H. SNYDER, OF SALT LAKE CITY, UTAH.

## PROCESS OF SEPARATING ZINC AND LEAD.

No Drawing.

Application filed November 24, 1919. Serial No. 340,219.

To all whom it may concern:

Be it known that I, EDWARD H. SNYDER, a citizen of the United States, residing at Salt Lake City, in the county of Salt Lake and State of Utah, have invented certain new and useful Improvements in Processes of Separating Zinc and Lead, of which the following is a specification.

The present invention has for its object 10 to separate and recover as separate materials the lead and zinc components of ores containing both lead zinc, which ores may also contain other metals in useful quantities. It has for a long time been recognized that 15 the lead present in zinc ores is objectionable in some of the processes of making zinc, and the zinc present in lead ores is objectionable in some of the processes of producing lead, the two metals each acting to render more 20 difficult the extraction of each other from the ores. Processes have been proposed heretofore for separating the two metals, or separately recovering the two metals from such ores, but these processes all have more 25 or less drawbacks.

The present invention is directed to a process in which both the lead and zinc are fumed off from the ore in the form of compounds, and the fume is so collected that it 30 contains large quantities of lead sulfate and zinc oxid. This operation may conveniently be accomplished in known manner, for example by the process of U. S. Patent No. 1,276,058 issued to R. G. Hall. The present 35 invention embraces the treatment of the fume or bag-house product of the Hall process, in such a way as to separate, as completely as possible, the lead from the zinc. The bag-house product produced in accordance 40 with the Hall process consists largely of lead sulfate and zinc oxid. An analysis of a typical example of the said bag-house product is as follows:

|                                               |       |
|-----------------------------------------------|-------|
| 45 Zinc oxid-----                             | 72%   |
| Lead sulfate-----                             | 20%   |
| Silica-----                                   | 3%    |
| Sulfur as sulfide-----                        | trace |
| 50 Other metal oxids, alumina and carbon----- | 5%    |

This product constitutes a concentrate of the lead and zinc contents of the ore under treatment and exists in a finely-divided and more or less fluffy condition. It is, after 55 collection, first mixed with finely crushed salt (sodium chlorid) and in this operation it

is essential to get a thorough distribution of the salt through the mass. It is advisable to first thoroughly mix the materials dry and then to add only a small quantity of water, 60 after which the product can be dried in suitable manner, and comminuted if desired. The mass is then fed into a furnace in which it is heated in an oxidizing atmosphere to a temperature at which the lead volatilizes in the 65 form of chlorid substantially completely from the mixture, leaving the bulk of the zinc oxid unchanged. It will accordingly be obvious that an amount of sodium chlorid chemically equivalent to the lead present, or 70 in practice an excess of this quantity, should be employed. Under these conditions no substantial quantity of the zinc is chloridized. The lead chlorid begins volatilizing at a temperature at about 750° C., and in order 75 to accomplish the complete volatilization of the lead as chlorid, it is necessary to carry the temperature up to about 1000 to 1100° C. As above stated, this operation must be conducted in an oxidizing atmosphere, or else 80 zinc will also be volatilized as chlorid. The lead chlorid fume is collected from the gases in any suitable manner, for example, by bag filters, Cottrell precipitators or in any other known manner, and the lead chlorid thus 85 collected can be converted into pig lead, lead salts, pigments or used for any other desired purposes. Certain other metals which may be present in the mass will, to some extent, 90 also volatilize and may be recovered or separated in known manner.

The furnaced residue contains zinc oxid quite free from lead and may be at once reduced to spelter, or employed for various other purposes. Zinc oxid, which is free 95 from lead, brings a considerably higher price than leaded zinc oxid containing the same amount of zinc.

The heating and chloridizing operation 100 can be carried out in any suitable form of furnace, for example a straight line mechanically or hand rabbled reverberatory furnace can be used for this purpose. If gas is available as fuel, the muffle type roaster similar to those employed for making sulfuric acid from zinc sulfide ores, can 105 be employed. This type of furnace has the advantage that the products of combustion do not mix with the gas carrying the lead chlorid fume, thereby reducting the volume 110 of gas to be handled in the treaters employed for collecting the lead fume. In this opera-

tion a small current of air is admitted to the muffles in order to insure the maintenance of the oxidizing atmosphere. Any zinc chlorid which is formed during the roasting 5 operation is largely converted back into zinc oxid and chlorine or hydrochloric acid so that very little of the zinc goes into the lead fume. The amount of zinc lost from the charge during the chloridization operation 10 is very small, due to the following facts:

I. Zinc oxid does not decompose sodium chloride to any appreciable extent in a neutral or oxidizing atmosphere at temperatures up to white heat.

15 II. Zinc chlorid, even if formed in a chloridizing roast, in the presence of air, is largely reconverted into zinc oxid, which is non-volatile.

III. The zinc in the product going into 20 chloridization furnace contains substantially the whole of its zinc in the form of oxid.

IV. The lead in the bag-house product subjected to chloridization exists practically 25 entirely in the form of sulfate which salt is capable of reacting with sodium chlorid to form lead chlorid.

V. Lead chlorid volatilizes readily and without decomposition at temperatures between 750 and 1100° C., (or better between 30 800 and 1100° C.), and can be collected from the gases substantially quantitatively.

It is to be understood that sodium chlorid is above referred to as being in most localities the cheapest and most convenient halogen salt to employ. In some locations, it may be advisable to employ other halogen salts of alkali-forming metals, thus calcium chlorid can be employed if desired.

I claim:

40 1. A process which comprises roasting lead-zinc ore containing sulfur and thereby making a product containing large quanti-

ties of lead sulfate and zinc oxid, intimately mixing such product with a chlorid of an alkali-forming metal in amount at least 45 chemically equivalent to the lead compound present in the product, and heating the mass in a non-reducing atmosphere to a temperature between 750° C., and 1100° C., whereby the lead is substantially converted into 50 chlorid and volatilized, and the zinc oxid remains substantially unvolatilized, whereby the lead chlorid may be collected separately from the zinc oxid.

2. In the treatment of zinc-lead metallurgical materials, the step of roasting the same mixed with a chlorid of an alkali-forming metal, in an oxidizing atmosphere, at a temperature at which the lead will be volatilized as chlorid, while the zinc remains unvolatilized.

3. The process which comprises mixing salt with a metallurgical product containing large amounts of zinc oxid and lead sulfate, and heating the said mixture in a current of oxidizing gases to a temperature over 750° C., whereby lead is chloridized and volatilized but zinc is not.

4. A process of separating zinc and lead which comprises converting the lead largely 70 into sulfate and converting the zinc largely into oxid, adding a chloride of an alkali-forming metal, heating the mixture under non-reducing conditions to above 750° C., whereby lead is volatilized substantially 75 without the volatilization of zinc, and collecting the lead fume.

In testimony whereof I affix my signature in the presence of two witnesses.

EDWARD H. SNYDER.

Witnesses:

OSCAR G. FUNKE,  
RALPH H. CAMERON.